

Patented Oct. 22, 1940

2,219,164

# UNITED STATES PATENT OFFICE

2,219,164

## EXTREME PRESSURE LUBRICANT

Franz Rudolf Moser, Amsterdam, Netherlands, and Marinus Cornelis Tuyn, Pladjo, Dutch East Indies, assignors to Shell Development Company, San Francisco, Calif., a corporation of Delaware

No Drawing. Application March 16, 1936, Serial No. 69,163. In the Netherlands March 19, 1935

6 Claims. (Cl. 252—48)

This invention relates to lubricants suitable for lubrication under extreme pressure conditions.

It is well known that the high pressures occurring in certain types of gears and bearings may cause a film of lubricant to rupture with consequent damage to the machinery. It has been shown that mineral lubricating oils can be improved with regard to their protective effect on rubbing surfaces by the addition of certain substances, so that excessive wear, scuffing and seizure, which normally follow a break in the film of lubricant, can thus be prevented even under the most unfavorable pressure and speed conditions. Oils possessing this highly desirable property are called extreme pressure lubricants.

We have discovered that members of the class of organic compounds containing the radical  $-\text{SO}_2\text{X}$ , in which X is a halogen, when added to mineral lubricating oils in relatively small quantities of the order of a few percent, are capable of imparting to the latter extreme pressure properties. The quantities of the compounds required never exceed 5% and in most instances 25 are 2% or less.

As examples of the organic compounds referred to, which may be aliphatic or cyclic, e. g. aromatic, and may contain substitution groups, such as  $-\text{NH}_2$ ,  $-\text{OH}$ ,  $-\text{COOH}$ , and halogen, methyl sulfochloride, methylene di-sulfochloride, ethyl sulfochloride, ricinoleic acid sulfochloride, benzene sulfochloride, benzene sulfofluoride, chlorbenzene sulfochloride, p-toluene sulfochloride, p-toluene sulfobromide, o-toluene sulfobromide, di-methyl aniline sulfochloride, anisol sulfochloride, phenetol sulfochloride, benzoic acid sulfochloride, di-phenyl sulfochloride, di-phenyl oxide sulfochloride, salicilic acid sulfochloride, benzidin sulfochloride, naphthalene sulfochloride, naphthol sulfochlorides, naphthylamine sulfochlorides, naphthalene di-sulfochlorides, amino naphthol di-sulfochlorides, anthracene sulfochloride, anthraquinone sulfochloride, alizarin sulfochloride, amido anthraquinone sulfochloride, may be mentioned.

Normally we prefer to use compounds of the organic sulfohalide group because, besides being highly effective in the matter of imparting extreme pressure properties to lubricants, most of them are readily soluble in effective concentrations in lubricating oils, thermally stable up to 200° C. and remarkably resistant to hydrolysis. For instance, p-toluene sulfochloride which is a by-product in the manufacture of saccharin, can be boiled with water for hours without apparent sign of decomposition. Also  $\beta$ -naphthalene sulfochloride and p-toluene sulfobromide may be used advantageously.

Compounds, which have a tendency to hydrolyze under operating conditions, may be used

to advantage in combination with corrosion inhibitors and it is generally good practice to use corrosion inhibitors in combination with our compounds, because under some circumstances, for instance, due to contact with decomposition catalysts, such as certain metals, even the more stable ones may develop some degree of corrosiveness. Efficient corrosion inhibitors which are effective in small quantities are the high molecular weight poly-carboxylic acids of the type described in the Moser application, Serial No. 12,247, filed March 21, 1935, nitrogen bases of the quinoline type, petroleum bases, poly-hydrocromatic compounds, and oil-soluble pickling inhibitors, in general.

Compounds of the group hereinbefore described are superior in the matter of imparting extreme pressure properties to other compounds also containing sulfur and halogen but not in the form of the  $-\text{SO}_2\text{X}$  radical. For instance, it was found that the methyl ester of p-chlorbenzene sulfonic acid, or the chlorehethyl ester of benzene sulfonic acid, barely raises the load carrying capacity of a lubricating oil to which they are admixed, while an equal amount of a compound of our group such as p-toluene sulfochloride, which has the same ultimate composition as the methyl ester of p-chlor benzene sulfonic acid, raises the extreme pressure property of the lubricating oil beyond the welding pressure range of the instrument used for testing. The instrument was the four-ball apparatus described in "Engineering" vol. 136 (1933) p. 46; this apparatus is capable of measuring the comparative metal wear at various pressures, as well as the pressures at which the test metals weld in the presence of the test lubricants.

Comparative typical experimental data obtained with the four-ball apparatus are given below:

| Substance added                  | Percent | Welding press. in kg. | Diameter wearing surface in mm. |    |
|----------------------------------|---------|-----------------------|---------------------------------|----|
| Straight mineral                 |         | 150                   | 2.2 at 100 kg.                  |    |
| p-Toluene sulfochloride          | 5       | 350                   | 2.29 at 300 kg.                 | 45 |
| Do                               | 1.0     | 500                   | 1.69 at 400 kg.                 |    |
| Do                               | 2.0     | Above 600             | 1.53 at 600 kg.                 |    |
| o-Toluene sulfochloride          | 2.0     | Above 600             | 1.79 at 600 kg.                 |    |
| p-Toluene sulfobromide           | 2.0     | Above 600             | 1.58 at 600 kg.                 |    |
| Methyl sulfochloride             | 2.0     | Above 600             | 1.60 at 600 kg.                 |    |
| Methylene disulfochloride        | 2.0     | Above 600             | 1.65 at 600 kg.                 |    |
| Chlorobenzene sulfochloride      | 2.0     | Above 600             | 1.67 at 600 kg.                 |    |
| Methyl p-chlorbenzene-sulfo-nate | 2.0     | 200                   |                                 | 50 |
| Chlorehethyl benzene-sulfonate   | 2.0     | 200                   |                                 |    |

The usefulness of the compounds hereinbefore described is not restricted to blends with lubricating oils alone, but extends to greases and other compounded lubricants as well. Where moisture-containing and/or alkaline reacting lubricants, such as soda or lime soap greases, are to be converted into extreme pressure lubricants, we

prefer using those compounds of the group which are not subject to ready hydrolysis, e. g., sulfoxy and sulfohalides described hereinbefore.

We claim as our invention:

- 5 1. A lubricant comprising a predominating quantity of a mineral oil lubricant and a small quantity of a compound having the formula  $R(SO_2X)_m$  in which R is an aliphatic radical, m is one or two, and X is a halogen.
- 10 2. The lubricant of claim 1 in which the amount of the compound is not more than 5%.

3. The lubricant of claim 1 in which the amount of the compound is not more than 2%.

4. The lubricant of claim 1 in which the compound is methyl sulfochloride.

5. The lubricant of claim 1 in which the compound is methylene di-sulfochloride.

6. The lubricant of claim 1 in which the compound is ethyl sulfochloride.

FRANZ RUDOLF MOSER.

MARINUS CORNELIS TUYN.

10